# EUROPEAN PATENT SPECIFICATION

(11) **EP 4 493 020 B1**
(45) Date of publication and mention of the grant of the patent: **20.05.2026**
(21) Application number: 23708911.5
(22) Date of filing: 22.02.2023
(51) Int. Cl.: A44C 27/00, A01K 61/56, A44C 17/00

(54) **PROCESS FOR THE PRODUCTION OF PEARLS BASED ON SEA WATER AND EPOXY RESIN, KIT OF MOLDS AND PRODUCT THUS OBTAINED**
VERFAHREN ZUR HERSTELLUNG VON PERLEN AUF BASIS VON MEERWASSER UND EPOXIDHARZ, FORMKIT UND SO ERHALTENES PRODUKT
PROCÉDÉ DE PRODUCTION DE PERLES À BASE D'EAU DE MER ET DE RÉSINE ÉPOXY, KIT DE MOULES ET PRODUIT AINSI OBTENU

(30) Priority: 17.03.2022 IT 202200005222
(43) Date of publication of application: 22.01.2025
(73) Proprietor: Perle dell'Elba S.r.l.s., 57034 Campo nell'Elba (LI) (IT)
(72) Inventor: BOCCIA, Elisa, 57034 Campo nell Elba (LI) (IT)
(74) Representative: Fiammenghi, Eva
(86) International application number: PCT/IB2023/051595
(87) International publication number: WO 2023/175415

(56) References cited:
- EP-A1- 3 750 399
- EP-A1- 3 804 554
- WO-A1-2020/079940
- JP-A- 2007 195 808
- JP-A- H06 245 667
- US-A1- 2009 090 133

## Description

### Field of the invention

The present invention relates to the field of jewelry and fashion. More specifically, within this field of the industry, the invention described and claimed below specifically relates to an innovative method, characterized by the use of sea water as a complementary component to the two-component epoxy resin, managing to keep the catalysis process and thus the solidification process intact, transforming the sea water itself from a liquid state to a solid state and creating wearable pearls.

### Prior art

Two-component resins are thermosetting polymers with cold reaction. The formulation is normally made up of a base resin (component A) and a hardener (component B), which, mixed carefully in the ratio indicated by the manufacturer, solidify, giving rise to a glossy vitrified layer.

Resins, mainly epoxy resins, are used in various fields, from construction to the electronics industry, as well as in the automotive, nautical and aeronautical fields, but also for the creation of various kinds of products in the fashion sector. One of the features of the resins is the absolute "iticoinpitibility" towards humidity and obviously even more than water, which makes them unusable, as it does not allow their catalysis and therefore the impossibility of the solidification process.

In fact, until now, resins are used to coat or incorporate only solid or dried objects or materials.

In the fashion sector, there are many lines of jewels made with resins, but they exclusively involve the use of resin alone with plays of color (through the use of specific dyes mainly in powder form) or with more or less precious stones incorporated therein.

There are a variety of websites offering resin purchasing choices specifically targeted at the production of "jewelry" and costume jewelry products such as www.kustomservice.com which offers a "clear fast drying cast epoxy for creating jewels, bracelets and bijoux". Among other things, there do not seem to be any patents in this regard yet. Up to now, a resin capable of solidifying by interacting with a substantial aqueous component that would allow the production of jewels has never been used on the market. In the present case, the object of the present patent application for an industrial invention is to create a method of producing long-lasting pearls, the result of a compound which represents a complete innovation in the sector, which can be made in a plurality of colors, creating a product resulting from an experiment drawn from the experience in the field of jewelry, craftsmanship and ingenuity. WO2020/079940A1 discloses a process for the production of epoxy pearls, a mold for said process and pearls obtained therefrom.

### Description of the invention

According to the present invention, a method is described for producing pearls, consisting of epoxy resin and sea water, resistant to external agents and able to last over time which effectively solves the above drawbacks.

The idea on which the project is based was to "materially" bring a natural element, precious for the human species, into a wearable jewel, replacing the traditional sea pearl with a product obtained from sea water itself.

The most advantageous feature consists in the design of a process which, by combining salt water as a complementary component to the two-component epoxy resin, manages to keep the catalysis process, therefore of solidification, intact.

The pearls in question are thus mainly made up of sea water mixed with epoxy resin in component A and component B, catalyst of the first component A and corn starch, alcohol dye for epoxy resins. This composition makes them resistant over time to both external agents and stress.

For the creation of pearls, the production method takes place in several steps as listed below and then described in detail:
(a) collecting sea water;
(b) filtering:
(c) boiling;
(d) mixing sea water, component A epoxy resin, corn starch, dye for epoxy resins and resting the mixture;
(e) adding component B epoxy resin;
(f) heating the compound, mixing and resting in immersion (bain-marie) for 6 minutes in hot water at about 40 °C;
(g) casting in a first mold;
(h) crystallizing the compound for about 36/48 hours until solidification;
(i) cleaning, smoothing and matting;
(j) "covering" in a second mold and addition of two-component epoxy resin;
(k) polishing and completion.

The initial step is that of collecting the sea water, which is carried out using a common non-toxic food-grade polyethylene receptacle with a capacity of 3 liters. Subsequently the water is filtered with a simple funnel with a mesh filter of variable size, brought to the boil for about 15 seconds in a first steel container and then, once cooled, decanted into a second glass container of 0, 75 liters. At the end of step (b) and of step (c) the sea water is ready to be processed and crystallized.

The next step is the one in which the crystallization process takes place and in which the aforementioned additional ingredients will be needed, in addition to the previously prepared sea water: in fact, in a third container, the processed sea water, a predefined quantity of epoxy resin in component A is added which condensate, the sea water, thanks also to corn starch. At the same time, a predefined quantity of alcohol dye for epoxy resins is mixed with the aforementioned elements to uniform the natural whitish color due to the crystallization of the sea salt present in the sea water. The aforementioned mixing of said substances added in said third container takes place by means of at least a small spatula or any other instrument, preferably made of wood or steel, to amalgamate the compound thus obtained. A 15-minute wait is necessary to allow for the elimination of any presence of air created following mixing. Subsequently, the aforementioned component B is added to the compound obtained so far in the aforementioned third container to catalyze the previously added epoxy resin. At this stage the mixture is immersed (bain-marie), inside said third container, in water heated to 40°C and mixed again for 2 minutes. Once a homogeneous consistency is reached, the mixture is left to rest in immersion (bain-marie) in the same hot water, for about 6 minutes. Optionally, this last step can be replaced by the use of a degasser machine which speeds up the elimination of the air bubbles generated by the mixing.

This is followed by the step dedicated to modeling the compound, which is first poured into a first mold: here the compound is distributed in spherical or other shaped impressions, included in the matrix of a special mold, with a diameter between 7 mm and 17mm. Furthermore, the mold comprises at least a centering pin, two feed tubes with a diameter between 3 mm and 5 mm and at least an air vent tube to allow the crystallization of the compound. The completion of the crystallization takes place in a time of about 36/48 hours when, once completely solidified, a first stage of raw pearls is obtained which are thus extracted from the impressions. In the following steps, it is necessary to remove the excess parts on the external surface: this step takes place inside a vibrating tumbler which, using abrasive coties, smooths and dulls the pearls in 45 minutes.

Subsequently, inside a plurality of second impressions of dimensions greater by about 1 mm than those previously used, and included in a second mold, two-component, transparent epoxy resin is poured again, filling each impression approximately halfway. This is the "covering" step during which the polished pearls are inserted into the aforementioned second impressions containing the epoxy resin and left to rest for a further 36/48 hours. Thus, advantageously, a layer of protective film of 0.5 mm is created on the entire external surface of each bead, eliminating any imperfections, irregularities and guaranteeing a greater brightness of the final product which is finally extracted from the second mold and polished, thanks to a goldsmith's polishing wheel which, with special cotton brushes and polishing waxes, also completes the outermost layer of the seawater pearls.

In a further advantageous version, in the aforementioned mixing step (d), 10 g of said component A epoxy resin are poured into the aforementioned third container, 0.25 g of corn starch are added, in 1.5 g of boiled sea water and a white alcohol drop for epoxy resins, which uniforms the natural whitish color due to the crystallization of the sea salt contained in sea water.

Always in a further and advantageous version in the above-mentioned mixing step (d) the alcohol-based colorant for epoxy resins is added alternatively in a blue tone and/or in other versions of a different color, following the same processing steps and the same crystallization procedure of the sea water salt using ½ drops of dye directly inside said first mold.

Advantageously in step (e) the epoxy resin catalyst component B is added following a ratio of 100:66 with respect to the amount of epoxy resin component A.

Possibly and advantageously, said first mold is made of steel while the second mold is made of silicone so as to allow the beads to be extracted once they have been covered without risking damaging their surface, even if only slightly.

In addition to the white edition, there are blue colors and/or a plurality of variants. Furthermore, in a plurality of variants, each collection is provided with different models that include author's ornaments, creation of unique pieces of collections or customizations requested by clients.

The result is advantageously a jewel that has, therefore, a great resistance over time, thanks to the raw material, and as already mentioned to the alcohol color, which penetrates the resin and blends together homogeneously.

In further versions the models include:
- bead covers in silver/gold or other metals for making pendants for necklaces, bracelets, earrings, brooches, key rings and other models relating to the jewelry sector,
- bead cover in silver/gold or other metals, in the shape of the island of Elba for making a pendant for a necklace,
- bead cover in silver/gold or other metals in the shape of the island of Elba to make a bracelet,
- bead cover in silver/gold or other metals in the shape of the island of Elba to make earrings,
- bead cover in silver/gold or other metals in the shape of the island of Elba to make key chains,
- bead cover in silver/gold or other metals in the shape of the island of Elba to make brooches,
- ring in silver/gold or other metals with white, blue pearl and/or in a plurality of other colors of your choice.

The advantages offered by the present invention are clear in the light of the above description and will be even clearer from the accompanying figures and the related detailed description.

### Description of the figures

The invention will hereinafter be described in at least a preferred embodiment thereof by way of non-limiting example with the aid of the accompanying figures, in which:
- FIGURE 1 illustrates the flow chart of the steps comprised in the process of the present invention from (a) to (k). Note that the sea water 110 of step (a) gradually changes to become a compound 110.4 with the addition of component A and component B epoxy resin 111.A, 111.B, corn starch 112 and alcohol dye 113.
- FIGURE 2 shows a view of the first mold 200 used in step h for shaping the beads 100 in question. Note the matrix 206 which mainly comprises a plurality of spherical impressions 201, of increasing diameter, at least a centering pin 203, feeding tubes 204 and air venting tubes 205.

### Detailed description of the invention

The present invention will now be described purely by way of non-limiting or binding example with the aid of the figures, which illustrate some embodiments relative to the present inventive concept.

With reference to FIG. 1 shows the steps of the process aimed at the production of pearls 100, constituted by epoxy resin 111 and sea water 110 resistant to external agents and stresses so as to last over time which constitutes the present invention.

The steps that make up this method are described below:
An initial step (a): during this step sea water 110 is collected, necessary in all the subsequent steps of the process through the use of a non-toxic polyethylene container 140 for food or through any other means for collecting liquids; the capacity of the container 140 is preferably of a flow rate of 3 liters.

Subsequently, once the necessary sea water 110 has been collected, still to be purified, the preparation steps of the same start, divided into:
b. a filtration step which occurs through a funnel 120 comprising a metal filter 130 with meshes of variable size;
c. a boiling step of the freshly filtered sea water 110.1 through the use of a first container 150, which is preferably made of steel, to be positioned in contact with a heat source for the elimination of any impurities naturally present in the collected liquid.

Subsequently, the boiled sea water 110.2 is transferred into a second container 160 having a capacity of at least 0.75 liters and preferably made of glass to be kept before the subsequent steps.

This is followed by a step (d) during which boiled sea water 110.2 is added to a third container 170 made of glass, plastic and/or any other material (the following proportions refer to a quantity of water of 1.5 g): 10 g of epoxy resin component A 111.A, 0.25 g of corn starch, 1-2 drops of white alcohol dye for epoxy resins 113 which makes the natural whitish color uniform due to the crystallization of the sea salt present in the water of sea. The aforementioned alcohol dye 113 is alternatively added in blue tones and/or in other color versions, following the same processing steps and the same crystallization procedure.

The step of mixing of said substances added in said third container 170 takes place by means of at least a small spatula or any other instrument, preferably made of wood or steel, to obtain a compound 110.3. Once mixing has taken place, there is a predefined time delay, preferably 15 minutes, to eliminate any presence of air created as a result of said mixing. Subsequently, in step (e), a component B 111.B, the catalyst of the aforementioned epoxy resin, is combined with the compound 110.3 obtained so far in a predetermined quantity, preferably in a 100:66 ratio with respect to the quantity of the aforementioned component A epoxy resin 111.A or on the basis of the quantitative ratios indicated in each resin used. Step (f): the aforementioned third container 170 is immersed in water (bain-marie) previously heated to a temperature of approximately 40°C, to heat the aforementioned compound 110.4, once the catalyst has been added, which is mixed again for at least 2 minutes. Once a homogeneous consistency has been reached, the compound 110.4 is left to rest, for approximately 6 minutes, in immersion (bain-marie) in the same water at 40°C. As an alternative to the practice of immersion, the process object of the present invention can provide for the use of a degasser machine capable of eliminating the air bubbles created by mixing.

Once the mixing steps have been completed, step (g) starts in which the compound 110.4 is poured into at least a first mold 200, preferably made of steel, which provides a matrix 206 comprising spherical impressions 201 of increasing diameter (variable) from the most small to the largest, from 7 mm to 17 mm, at least a centering pin 203, at least two feeding tubes 204 with a diameter between 3 mm and 5 mm, at least an air venting tube 205.

In the following 36/48 hours, there is a step (h) of waiting for the crystallization of the compound containing sea water 110.4 until complete solidification and the obtainment of raw pearls 100. At the end of this step each of the beads 100 is extracted from the aforementioned first mold 200 to then be finished in step (i). At first, in fact, each of the pearls 100 is cleaned on the external surface, with the use of abrasive files any protrusions and excess parts are removed. Immediately afterwards they are inserted into a vibrating tumbler, having abrasive cones inside, preferably for 45 minutes. Here the pearls 100 are smoothed and opacified.

The next step (j), of "covering", takes place in a second mold 210 having second spherical impressions 202 with a diameter greater than the previous ones by approximately 1 mm:
- approximately half of each spherical impression 202 is filled with transparent two-component epoxy resin 111.A, 111.B, to be mixed in predetermined proportions based on the ratio indicated by the manufacturer of the resin used;
- insertion of the aforementioned polished and opaque beads 100 into the second spherical impressions 202 containing epoxy resin 111;
- rest for an interval of time between 36/48 hours aimed at allowing the creation of a layer of protective film of 0.5 mm on the external surface of each pearl 100. This layer of protective film, in addition to eliminating any imperfections, guarantees greater brightness to the final product and greater resistance to external agents.

In the final step (k) the pearls 100 are extracted from the aforementioned second mold, polished, by means of a goldsmith's polishing wheel having cotton brushes and suitable polishing waxes, until completion of the production process.

The pearls 100 thus produced can be made as a single piece, as part of a collection, distinguished by the same graphic reproduction, in a plurality of different models, shapes and colors, with silver/gold or other metal bead caps and for making bracelets, necklaces, earrings, rings, key rings, brooches, cufflinks, or other models related to the jewelry sector, wearable or for display.

Finally, it is clear that modifications, additions or variants may be made to the invention described thus far which are apparent to those skilled in the art, without departing from the scope of protection that is provided by the appended claims.

## Claims

1. A process for the production of pearls (100) obtained from an epoxy resin (111) and sea water (110), which resist to external agents and are durable, wherein these pearls (100) are adapted for the manufacture of any kind of jewel to be exhibited and/or wearable, are realizable in one piece, as part of a collection, and are distinguishable through the same graphic reproduction on customer request, the process being **characterized in that** it comprises the following steps:
(a) collecting sea water (110) with at least a receptacle made of non-toxic food-grade polyethylene (140) which has a capacity of 3 liters, or by any other means suitable for collecting water, said step (a) being apt to provide raw material for the manufacture of said pearls (100);
(b) filtering said sea water (110), using a funnel (120) with a first and a second end, the second end comprising at least a filter (130) made of metal having meshes of variable size;
(c) boiling the filtered sea water (110.1), using at least a first preferably steel-made container (150), adapted for bringing to boil said filtered sea water (110.1) when put in contact with a heat source in order to eliminate any impurity; wherein this processing step (c) uses at least a second container (160), or any other container preferably made of glass and with a capacity of at least 0.75 liters; wherein said second container (160) is adapted for containing said boiled sea water (110.2) following said filtering and boiling steps;
(d) mixing said boiled sea water (110.2) using at least a third glass made or plastic made container (170), and/or a container made of any other material while adding the following:
• an epoxy resin (111) divided into component A (111.A) and component B (111.B) acting as an epoxy resin catalyzer;
• corn starch (112);
• alcohol based stain for epoxy resins (113);
specifically, adding initially said boiled sea water (110.2) into said third container (170), a predefined quantity of said epoxy resin component A (111.A) capable of condensing said sea water (110) in combination with said corn starch (112), and a predefined quantity of said alcohol based stain for epoxy resins (113) suited to homogenize the natural whitish color due to a crystallization of the sea salt present in said sea water (110.2) processed up to now; wherein said mixing of substances added to said third container (170) is performed by means of at least a spatula or of any other tool, preferably made of wood or steel, adapted for mixing the composite material (110.3) obtained in this manner; wherein, the above is followed by a predefined waiting time, preferably of 15 minutes, for eliminating the possible presence of air created as a consequence of said mixing;
(e) adding said epoxy resin catalyzing component B (111.B) in a predefined amount to said composite material (110.3) in said third container (170);
(f) submerging said third container (170) containing said composite material (110.4) as obtained till now, in preheated water, preferably at about 40°C, mixing for about 2 minutes by means of said spatula, until a homogeneous consistency is obtained for the catalyzed composite material (110.4), and leaving the same immersed in this warm water for about 6 minutes; wherein, as an alternative to step (f) a degassing machine is used, which is adapted for removing the air bubbles caused by the mixing;
(g) casting of said composite material (110.4) in at least a first mold (200), wherein said first mold (200) includes a plurality of impressions (201) of increasing diameters, from the smallest to the greatest one;
(h) waiting for the completion of the crystallization of said composite material (110.4), preferably for about 36/48 hours, until a complete solidification is achieved and raw pearls (100) are obtained; removal/extraction of said pearls (100), in a raw condition, from said impressions (201);
(i) a cleaning step, for cleaning the pearls (100), by removing possible excess parts with abrasive files and introduction of the pearls in a vibrating tumbler for a period of preferably 45 minutes; wherein said tumbler internally includes abrasive cones apt to polish, to dull and to prepare said pearls (100) for a subsequent covering step with a "shell";
(j) said pearls (100) are introduced in a second mold (210) comprising second impressions (202) whose diameter exceeds by about 1 mm the diameter of the respective first impressions (201) employed in said crystallization step; wherein, said impressions (202) are filled halfway or so, with a transparent two-component epoxy resin (111.A, 111.B) mixed in predetermined ratios, according to the ratio indicated by the manufacturer of the resin used during this covering step; wherein, upon polishing and dulling, said pearls (100) are introduced in said second impressions (202) containing the epoxy resin; wherein during a further standing time of 36/48 hours, a layer of 0.5 mm thick protective film is allowed to form on the entire outer surface of said pearls (100); wherein, said layer of protective film eliminates possible imperfections, ensures an improved glossiness for the end product, and a greater resistance to external agents;
(k) extraction/removal of said pearls (100) from said second mold, polishing, by means of a goldsmith's polishing wheel comprising appropriate cotton brushes and appropriate polishing waxes for the finishing of said pearls (100).

2. A process for the production of pearls (100) obtained from an epoxy resin (111) and sea water (110), according to the preceding claim 1, **characterized in that** in the above step (d), 10 g of said epoxy resin component A (111) are poured in said third container (170), 0,25 g of corn starch are added to 1.5 g of said boiled sea water (110.2) together with a drop of alcohol based white stain for epoxy resins (113), adapted for homogenizing the natural whitish color due to said crystallization of the sea salt naturally contained in the sea water.

3. A process for the production of pearls (100) obtained from an epoxy resin (111) and sea water (110), according to the preceding claims 1 or 2, **characterized in that** in the above mixing step (d), the alcohol based stain for epoxy resins (113) is alternatively added in a shade of blue and/or in other shades of different color, and following identical processing steps and the same crystallization process of said sea water, by employing a resins' stain of various shades, according to the needs, which is added in an amount of 1-2 drops directly into said first mold (200) following said first casting.

4. A process for the production of pearls (100) obtained from an epoxy resin (111) and sea water (110), according to anyone of the preceding claims, **characterized in that** in the above step (e), said epoxy resin catalyzing component B (111.B) is added according to a ratio of 100:66, with respect to the amount of said epoxy resin component A (111.A).

5. A kit of molds for the manufacturing of pearls (100) obtained from epoxy resin (111) and sea water (110), **characterized in that** it comprises at least a steel-made first mold (200) and at least a second mold (210) made of silicone; wherein, said first mold (200) comprises a plurality of impressions or recesses (201) of increasing size from the smallest to the greatest one, adapted for use in a manufacturing process of pearls (100) according to the preceding claim 1, step (g); wherein, said second mold (210) comprises second impressions or recesses (202) having a size exceeding by about 1 mm said first impressions (201); wherein, said second mold (210) is adapted for being used in a manufacturing process of pearls (100), according to the preceding claim 1, step (j).

6. A kit of molds for the manufacturing of pearls (100) obtained from epoxy resin (111) and sea water (110), according to the preceding claim 5, **characterized in that** said steel made first mold (200) comprises a matrix (206) equipped with:
- impressions (201) inscribable in a diameter varying from 7 to 17 mm,
- a centering pin (203),
- feeding tubes (204) having a diameter between 3 mm and 5 mm,
- at least a venting tube for the air (205).

7. Pearls (100) constituted by epoxy resin (111) and sea water (110), obtained according to the process of claims 1 to 4 and been produced using the kit of claims 5 and 6, **characterized in that** they have a perfectly spherical shape of variable diameter, with an outer surface which is perfectly smoothed and polished.

8. Pearls (100) constituted by epoxy resin (111) and sea water (110), according to the preceding claim 7, **characterized in that** they are realized in a jewelry design/model that includes a pearl cover made of silver/gold or other metals, with the shape of the Elba Island, for obtaining a pendant for necklace and/or a bracelet and/or earrings and/or key holders, and/or brooches and/or other models/designs of the jewelry sector.

9. Pearls (100) constituted by epoxy resin (111) and sea water (110), according to anyone of the preceding claims from 7 onwards, **characterized in that** they are produced in a white edition model, apt to realize a ring made of silver and/or gold and/or other metals, with a white pearl.

10. Pearls (100) constituted by epoxy resin (111) and sea water (110), according to anyone of the preceding claims from 7 onwards, **characterized in that** they are produced in a blue edition model, apt to realize a ring made of silver and/or gold and/or other metals, with a blue pearl.

## Patentansprüche

1. Verfahren zur Herstellung von Perlen (100) aus einem Epoxidharz (111) und Meerwasser (110), die gegen äußere Stoffe beständig und langlebig sind, wobei diese Perlen (100) für die Herstellung jeder Art von Schmuckstück geeignet sind, um ausgestellt und/oder getragen zu werden, realisierbar sind in einem Stück, als Teil einer Kollektion und auf Kundenwunsch durch dieselbe grafische Darstellung unterscheidbar sind, wobei das Verfahren **dadurch gekennzeichnet ist, dass** es die folgenden Schritte aufweist:
(a) Sammeln von Meerwasser (110) mit zumindest einem Behälter aus ungiftigem, lebensmittelechtem Polyethylen (140), der ein Fassungsvermögen von 3 Litern aufweist, oder durch jedes andere Mittel, das zum Sammeln von Wasser geeignet ist, wobei der Schritt (a) dazu dient, Rohmaterial für die Herstellung der Perlen (100) bereitzustellen;
(b) Filtern des Meerwassers (110) unter Verwendung eines Trichters (120) mit einem ersten und einem zweiten Ende, wobei das zweite Ende zumindest einen Filter (130) aus Metall mit Maschen unterschiedlicher Größe aufweist;
(c) Kochen des gefilterten Meerwassers (110.1) unter Verwendung von zumindest einem ersten, vorzugsweise aus Stahl gefertigten Behälter (150), der dazu ausgelegt ist, das gefilterte Meerwasser (110.1) zu kochen, wenn er mit einer Wärmequelle in Kontakt gebracht wird, um etwaige Verunreinigungen zu beseitigen; wobei dieser Verarbeitungsschritt (c) zumindest einen zweiten Behälter (160) oder einen beliebigen anderen Behälter, vorzugsweise aus Glas gefertigt und mit einem Fassungsvermögen von zumindest 0,75 Litern, verwendet; wobei der zweite Behälter (160) dazu ausgelegt ist, das gekochte Meerwasser (110.2) nach den Filterungs- und Kochschritten aufzunehmen;
(d) Mischen des gekochten Meerwassers (110.2) unter Verwendung von zumindest einem dritten aus Glas oder aus Kunststoff hergestellten Behälter (170) und/oder einem aus einem beliebigen anderen Material hergestellten Behälter, während das Folgende hinzugefügt wird:
• ein Epoxidharz (111), unterteilt in eine Komponente A (111.A) und eine Komponente B (111.B), die als Epoxidharz-Katalysator wirkt;
• Maisstärke (112);
• alkoholbasierte Beize für Epoxidharze (113);
insbesondere Hinzufügen zunächst des gekochten Meerwassers (110.2) in den dritten Behälter (170), einer vordefinierten Menge der Epoxidharzkomponente A (111.A), die in der Lage ist, das Meerwasser (110) in Kombination mit der Maisstärke (112) zu kondensieren, sowie einer vordefinierten Menge der alkoholbasierten Beize für Epoxidharze (113), die geeignet ist, die natürliche weißliche Färbung aufgrund einer Kristallisation des in dem bisher verarbeiteten Meerwasser (110.2) vorhandenen Meersalzes zu homogenisieren; wobei das Mischen der in den dritten Behälter (170) hinzugegebenen Substanzen mittels zumindest eines Spatels oder eines anderen Werkzeugs, vorzugsweise aus Holz oder Stahl, das zum Mischen des auf diese Weise erhaltenen Mischmaterials (110.3) geeignet ist, durchgeführt wird; wobei auf das Vorstehende eine vordefinierte Wartezeit, vorzugsweise von 15 Minuten, folgt, um das mögliche Vorhandensein von Luft, die infolge des Mischens erzeugt wurde, zu beseitigen;
(e) Hinzufügen der Epoxidharz katalysierenden Komponente B (111.B) in einer vordefinierten Menge zu dem Mischmaterial (110.3) in dem dritten Behälter (170);
(f) Eintauchen des dritten Behälters (170), der das bisher erhaltene Mischmaterial (110.4) enthält, in vorgewärmtes Wasser, vorzugsweise bei etwa 40 °C, Mischen für etwa 2 Minuten mittels des Spatels, bis eine homogene Konsistenz für das katalysierte Mischmaterial (110.4) erreicht ist, und Eingetauchtlassen desselben etwa 6 Minuten lang in diesem warmen Wasser; wobei als Alternative zu Schritt (f) eine Entgasungsmaschine, die zum Entfernen der durch das Mischen verursachten Luftblasen ausgelegt ist, verwendet wird;
(g) Gießen des Mischmaterials (110.4) in zumindest eine erste Form (200), wobei die erste Form (200) eine Vielzahl von Vertiefungen (201) mit zunehmenden Durchmessern, von der kleinsten bis zur größten, aufweist;
(h) Abwarten des Abschlusses der Kristallisation des Mischmaterials (110.4), vorzugsweise etwa 36/48 Stunden, bis eine vollständige Verfestigung erreicht ist und Rohperlen (100) erhalten werden; Entnahme/Entfernung der Perlen (100) in einem Rohzustand aus den genannten (201);
(i) einen Reinigungsschritt zum Reinigen der Perlen (100) durch Entfernen möglicher überschüssiger Teile mit abrasiven Feilen und Einbringung der Perlen in eine Vibrationstrommel für einen Zeitraum von vorzugsweise 45 Minuten; wobei die Trommel im Inneren Schleifkegel enthält, die geeignet sind, die Perlen (100) zu polieren, zu mattieren und für einen nachfolgenden Beschichtungsschritt mit einer "Hülle" vorzubereiten;
(j) wobei die Perlen (100) in eine zweite Form (210) eingebracht werden, die zweite Vertiefungen (202) aufweist, deren Durchmesser den Durchmesser der jeweiligen in dem Kristallisationsschritt verwendeten ersten Vertiefungen (201) um etwa 1 mm übersteigt; wobei die Vertiefungen (202) etwa zur Hälfte mit einem transparenten Zweikomponenten-Epoxidharz (111.A, 111.B), das in vorgegebenen Verhältnissen gemischt ist, gefüllt werden, und zwar gemäß dem durch den Hersteller des in diesem Ummantelungsschritt verwendeten Harzes angegebenen Verhältnis; wobei die Perlen (100) nach dem Polieren und Mattieren in die das Epoxidharz enthaltenden zweiten Vertiefungen (202) eingebracht werden; wobei zugelassen wird, dass sich während einer weiteren Standzeit von 36/48 Stunden eine Schicht aus einem 0,5 mm dicken Schutzfilm auf der gesamten Außenfläche der Perlen (100) bildet; wobei die Schicht aus dem dicken Schutzfilm mögliche Unzulänglichkeiten beseitigt, einen verbesserten Glanz für das Endprodukt gewährleistet und eine höhere Beständigkeit gegen äußere Einflüsse gewährleistet;
(k) Entnahme der Perlen (100) aus der zweiten Form, Polieren mittels einer Goldschmiedepolierscheibe mit geeigneten Baumwollbürsten und geeigneten Polierwachsen zur Endbearbeitung der Perlen (100).

2. Verfahren zur Herstellung von Perlen (100) aus einem Epoxidharz (111) und Meerwasser (110) gemäß dem vorhergehenden Anspruch 1, **dadurch gekennzeichnet, dass** in dem obigen Schritt (d) 10 g der Epoxidharzkomponente A (111) in den dritten Behälter
(170) gegossen werden, 0,25 g Maisstärke zu 1,5 g des gekochten Meerwassers (110.2) zusammen mit einem Tropfen alkoholbasierter weißer Beize für Epoxidharze (113) hinzugefügt werden, die zum Homogenisieren der natürlichen weißliche Farbe aufgrund der Kristallisation des in dem Meerwasser natürlicherweise enthaltenen Meersalzes geeignet ist.

3. Verfahren zur Herstellung von Perlen (100) aus einem Epoxidharz (111) und Meerwasser (110) gemäß den vorhergehenden Ansprüchen 1 oder 2, **dadurch gekennzeichnet, dass** im vorhergehenden Mischschritt (d) die alkoholbasierte Beize für Epoxidharze (113) alternativ in einem Blauton und/oder in Tönen anderer Farbe hinzugefügt wird, und nach identischen Verarbeitungsschritten und demselben Kristallisationsprozess des Meerwassers durch
Verwenden einer Harzbeize verschiedener Farbtöne, je nach Bedarf, die nach dem ersten Gießen in einer Menge von 1-2 Tropfen direkt in die erste Form (200) gegeben wird.

4. Verfahren zur Herstellung von Perlen (100) aus einem Epoxidharz (111) und Meerwasser (110) gemäß einem der vorhergehenden Ansprüche, **dadurch gekennzeichnet, dass** in dem obigen Schritt (e) die Epoxidharz katalysierende Komponente B (111.B) gemäß einem Verhältnis von 100:66, bezogen auf die Menge der Epoxidharz-Komponente A (111.A),
zugegeben wird.

5. Formensatz zur Herstellung von Perlen (100) aus Epoxidharz (111) und Meerwasser (110), **dadurch gekennzeichnet, dass** er zumindest eine aus Stahl hergestellte erste Form (200) und zumindest eine aus Silikon hergestellte zweite Form (210) aufweist; wobei die erste Form (200) eine Vielzahl von Vertiefungen oder Aussparungen (201) umfasst, deren Größe von der
kleinsten zur größten zunimmt und die für die Verwendung in einem Herstellungsverfahren für Perlen (100) gemäß dem vorhergehenden Anspruch 1, Schritt (g) geeignet ist; wobei die zweite Form (210) zweite Vertiefungen oder Aussparungen (202) mit einer Größe, die die ersten Vertiefungen (201) um etwa 1 mm übersteigt, aufweist; wobei die zweite Form (210) dazu geeignet ist, in einem Herstellungsverfahren von Perlen (100) gemäß dem vorhergehenden Anspruch 1, Schritt (j) verwendet zu werden.

6. Formensatz zur Herstellung von Perlen (100) aus Epoxidharz (111) und Meerwasser (110), gemäß dem vorhergehenden Anspruch 5, **dadurch gekennzeichnet, dass** die
aus Stahl hergestellte erste Form (200) eine Matrix (206) aufweist, die ausgestattet ist mit:
- Vertiefungen (201), die in einem von 7 bis 17 mm variierenden Durchmesser beschriftet werden können,
- einem Zentrierstift (203),
- Zuführrohren (204) mit einem Durchmesser zwischen 3 mm und 5 mm,
- zumindest einem Lüftungsrohr für die Luft (205).

7. Perlen (100), die durch Epoxidharz (111) und Meerwasser (110) gebildet sind, erhalten gemäß
dem Verfahren der Ansprüche 1 bis 4 und hergestellt unter Verwendung des Satzes der Ansprüche 5 und 6, **dadurch gekennzeichnet, dass** sie eine perfekt kugelförmige Gestalt mit variablem Durchmesser aufweisen, mit einer Außenfläche, die perfekt geglättet und poliert ist.

8. Perlen (100), die durch Epoxidharz (111) und Meerwasser (110) gebildet sind, gemäß dem vorhergehenden Anspruch 7, **dadurch gekennzeichnet, dass** sie in einem
Schmuckdesign/Modell, das eine Perlenumhüllung aus Silber/Gold oder anderen Metallen in der Form der Insel Elba realisiert sind, um einen Anhänger für eine Halskette und/oder ein Armband und/oder Ohrringe und/oder Schlüsselanhänger und/oder Broschen und/oder anderer Modelle/Designs aus dem Schmuckbereich zu erhalten.

9. Perlen (100), die durch Epoxidharz (111) und Meerwasser (110) gebildet sind, gemäß einem der vorhergehenden Ansprüche ab 7, **dadurch gekennzeichnet, dass** sie in einer weißen
Ausführung hergestellt sind, geeignet, um einen Ring aus Silber und/oder Gold und/oder anderen Metallen mit einer weißen Perle zu realisieren.

10. Perlen (100), die durch Epoxidharz (111) und Meerwasser (110) gebildet sind, gemäß einem der vorhergehenden Ansprüche ab 7, **dadurch gekennzeichnet, dass** sie in einer blauen Ausführung hergestellt sind, geeignet, um einen Ring aus Silber und/oder Gold und/oder anderen Metallen mit einer blauen Perle zu realisieren.

## Revendications

1. Procédé de production de perles (100) obtenues à partir d'une résine époxy (111) et d'eau de mer (110), qui résistent aux agents externes et sont durables, dans lequel lesdites perles (100) sont adaptées pour la fabrication de tout type de bijou à exposer et/ou à porter, sont réalisables en une seule pièce, dans le cadre d'une collection, et sont distinguables par la même reproduction graphique sur demande du client, le procédé étant **caractérisé en ce qu'**il comprend les étapes suivantes :
(a) la collecte d'eau de mer (110) avec au moins un récipient composé de polyéthylène de qualité alimentaire non toxique (140) qui présente une capacité de 3 litres, ou par tout autre moyen adapté pour la collecte d'eau, ladite étape (a) étant apte à fournir une matière première pour la fabrication desdites perles (100) ;
(b) le filtrage de ladite eau de mer (110), à l'aide d'un entonnoir (120) avec une première et une seconde extrémité, la seconde extrémité comprenant au moins un filtre (130) composé de métal présentant des mailles de taille variable ;
(c) l'ébullition de l'eau de mer filtrée (110.1), en utilisant au moins un premier contenant de préférence composé d'acier (150), adapté pour porter à ébullition ladite eau de mer filtrée (110.1) lorsqu'elle est mise en contact avec une source de chaleur afin d'éliminer toute impureté ; dans lequel cette étape de traitement (c) utilise au moins un second contenant (160), ou tout autre contenant de préférence composé de verre et ayant une capacité d'au moins 0,75 litre ; dans lequel ledit second contenant (160) est adapté pour contenir ladite eau de mer bouillie (110.2) après lesdites étapes de filtration et d'ébullition ;
(d) le mélange de ladite eau de mer bouillie (110.2) à l'aide d'au moins un troisième contenant composé de verre ou composé de plastique (170), et/ou d'un contenant composé de tout autre matériau tout en ajoutant ce qui suit :
• une résine époxy (111) divisée en un composant A (111.A) et un composant B (111.B) agissant comme catalyseur de résine époxy ;
• de l'amidon de maïs (112) ;
• une teinture à base d'alcool pour résines époxy (113) ;
notamment, l'ajout initial de ladite eau de mer bouillie (110.2) dans ledit troisième contenant (170), d'une quantité prédéfinie dudit composant de résine époxy A (111.A) capable de condenser ladite eau de mer (110) en combinaison avec ledit amidon de maïs (112), et d'une quantité prédéfinie de ladite teinture à base d'alcool pour résines époxy (113) adaptée pour homogénéiser la couleur blanchâtre naturelle due à une cristallisation du sel marin présent dans ladite eau de mer (110.2) traitée jusqu'à présent ; dans lequel ledit mélange de substances ajoutées audit troisième contenant (170) est réalisé au moyen d'au moins une spatule ou de tout autre outil, de préférence composé de bois ou d'acier, adapté pour mélanger le matériau composite (110.3) obtenu de cette manière ; dans lequel ce qui précède est suivi d'un temps d'attente prédéfini, de préférence de 15 minutes, pour éliminer la présence éventuelle d'air créé à la suite dudit mélange ;
(e) l'ajout dudit composant catalysant de résine époxy B (111.B) en une quantité prédéfinie audit matériau composite (110.3) dans ledit troisième contenant (170) ;
(f) l'immersion dudit troisième contenant (170) contenant ledit matériau composite (110.4) tel qu'obtenu jusqu'à présent, dans de l'eau préchauffée, de préférence à environ 40 °C, en mélangeant pendant environ 2 minutes à l'aide de ladite spatule, jusqu'à obtenir une consistance homogène pour le matériau composite catalysé (110.4), et l'immersion de ce dernier dans cette eau tiède pendant environ 6 minutes ; où, en alternative à l'étape (f), une machine de dégazage est utilisée, qui est adaptée pour éliminer les bulles d'air causées par le mélange ;
(g) le moulage dudit matériau composite (110.4) dans au moins un premier moule (200), dans lequel ledit premier moule (200) inclut une pluralité d'empreintes (201) de diamètres croissants, de la plus petite à la plus grande ;
(h) l'attente de la fin de la cristallisation dudit matériau composite (110.4), de préférence pendant environ 36/48 heures, jusqu'à ce qu'une solidification complète soit atteinte et que des perles brutes (100) soient obtenues ; l'élimination/l'extraction desdites perles (100), dans un état brut, à partir desdites empreintes (201) ;
(i) une étape de nettoyage, permettant de nettoyer les perles (100), en éliminant d'éventuelles parties excédentaires avec des limes abrasives et en introduisant les perles dans un godet vibrant pendant une période de préférence de 45 minutes ; dans lequel ledit godet inclut en interne des cônes abrasifs aptes à polir, à mater et à préparer lesdites perles (100) pour une étape de revêtement ultérieure avec une « coque » ;
(j) lesdites perles (100) sont introduites dans un second moule (210) comprenant des secondes empreintes (202) dont le diamètre dépasse d'environ 1 mm le diamètre des premières empreintes (201) respectives utilisées lors de ladite étape de cristallisation ; dans lequel lesdites empreintes (202) sont remplies à moitié ou presque avec une résine époxy transparente à deux composants (111.A, 111.B) mélangée dans des proportions prédéterminées, selon le rapport indiqué par le fabricant de la résine utilisée lors de cette étape de revêtement ; dans lequel, après le polissage et le matage, lesdites perles (100) sont introduites dans lesdites secondes empreintes (202) contenant la résine époxy ; dans lequel, durant un temps de repos supplémentaire de 36/48 heures, une couche de film protecteur de 0,5 mm d'épaisseur est laissée à former sur l'ensemble de la surface externe desdites perles (100) ; dans lequel, ladite couche de film protecteur élimine les éventuelles imperfections, assure un brillant amélioré pour le produit final et une plus grande résistance aux agents externes ;
(k) l'extraction/le retrait desdites perles (100) dudit second moule, le polissage, au moyen d'une meule de polissage d'orfèvre comprenant des brosses en coton appropriées et des cires de polissage appropriées pour la finition desdites perles (100).

2. Procédé de production de perles (100) obtenues à partir d'une résine époxy (111) et d'eau de mer (110), selon la revendication 1 précédente, **caractérisé en ce que** dans l'étape (d) ci-dessus, 10 g dudit composant de résine époxy A (111) sont versés dans ledit troisième contenant (170), 0,25 g d'amidon de maïs sont ajoutés à 1,5 g de ladite eau de mer bouillie (110.2) avec une goutte de teinture blanche à base d'alcool pour résines époxy (113), adaptée pour homogénéiser la couleur blanchâtre naturelle due à ladite cristallisation du sel marin naturellement contenu dans l'eau de mer.

3. Procédé de production de perles (100) obtenues à partir d'une résine époxy (111) et d'eau de mer (110), selon les revendications 1 ou 2 précédentes, **caractérisé en ce que** lors de l'étape de mélange (d) ci-dessus, la teinture à base d'alcool pour résines époxy (113) est alternativement ajoutée dans une teinte de bleu et/ou dans d'autres teintes de couleurs différentes, et suivant des étapes de traitement identiques et le même procédé de cristallisation de ladite eau de mer, en utilisant une teinture de résines de diverses teintes, selon les besoins, qui est ajoutée en une quantité de 1 à 2 gouttes directement dans ledit premier moule (200) suivant ledit premier moulage.

4. Procédé de production de perles (100) obtenues à partir d'une résine époxy (111) et d'eau de mer (110), selon l'une des revendications précédentes, **caractérisé en ce que** dans l'étape (e) ci-dessus, ledit composant catalyseur de résine époxy B (111.B) est ajouté selon un rapport de 100:66, par rapport à la quantité dudit composant de résine époxy A (111.A).

5. Kit de moules pour la fabrication de perles (100) obtenues à partir de résine époxy (111) et d'eau de mer (110), **caractérisé en ce qu'**il comprend au moins un premier moule composé d'acier (200) et au moins un second moule (210) composé de silicone ; dans lequel ledit premier moule (200) comprend une pluralité d'empreintes ou de creux (201) de taille croissante, de la plus petite/du plus petit à la plus grande/au plus grand, adapté(e)s pour une utilisation dans un procédé de fabrication de perles (100) selon la revendication 1 précédente, étape (g) ; dans lequel ledit second moule (210) comprend des secondes empreintes ou des seconds creux (202) présentant une taille dépassant d'environ 1 mm lesdites premières empreintes (201) ; dans lequel ledit second moule (210) est adapté pour être utilisé dans un procédé de fabrication de perles (100), selon la revendication 1 précédente, étape (j).

6. Kit de moules pour la fabrication de perles (100) obtenues à partir de résine époxy (111) et d'eau de mer (110), selon la revendication 5 précédente, **caractérisé en ce que** ledit premier moule composé d'acier (200) comprend une matrice (206) équipée des éléments suivants :
- des empreintes (201) inscriptibles avec un diamètre variant de 7 à 17 mm,
- une broche de centrage (203),
- des tubes d'alimentation (204) présentant un diamètre compris entre 3 mm et 5 mm,
- au moins un tube de mise à l'air (205).

7. Perles (100) constituées de résine époxy (111) et d'eau de mer (110), obtenues selon le procédé des revendications 1 à 4 et produites à l'aide du kit des revendications 5 et 6, **caractérisées en ce qu'**elles présentent une forme parfaitement sphérique de diamètre variable, avec une surface externe parfaitement lissée et polie.

8. Perles (100) constituées de résine époxy (111) et d'eau de mer (110), selon la revendication 7 précédente, **caractérisées en ce qu'**elles sont réalisées dans un design/modèle de bijou qui inclut un revêtement de perle composé d'argent/or ou d'autres métaux, présentant la forme de l'île d'Elbe, pour obtenir un pendentif pour collier et/ou un bracelet et/ou des boucles d'oreilles et/ou des porte-clés, et/ou des broches et/ou d'autres modèles/designs du secteur de la bijouterie.

9. Perles (100) constituées de résine époxy (111) et d'eau de mer (110), selon l'une des revendications précédentes à partir de la revendication 7, **caractérisées en ce qu'elles** sont produites dans un modèle d'édition blanc, permettant de réaliser une bague composée d'argent et/ou d'or et/ou d'autres métaux, avec une perle blanche.

10. Perles (100) constituées de résine époxy (111) et d'eau de mer (110), selon l'une des revendications précédentes à partir de la revendication 7, **caractérisées en ce qu'elles** sont produites dans un modèle d'édition bleu, permettant de réaliser une bague composée d'argent et/ou d'or et/ou d'autres métaux, avec une perle bleue.
